



US006139909A

# United States Patent [19]

Hagewiesche

[11] Patent Number: 6,139,909

[45] Date of Patent: \*Oct. 31, 2000

[54] **USING HYDROCARBON STREAMS TO PREPARE A METALLIC PROTECTIVE LAYER**

[75] Inventor: **Daniel P. Hagewiesche**, Oakland, Calif.

[73] Assignee: **Chevron Chemical Company**, San Francisco, Calif.

[\*] Notice: This patent issued on a continued prosecution application filed under 37 CFR 1.53(d), and is subject to the twenty year patent term provisions of 35 U.S.C. 154(a)(2).

[21] Appl. No.: **08/742,282**

[22] Filed: **Oct. 31, 1996**

## Related U.S. Application Data

[63] Continuation of application No. 08/475,308, Jun. 7, 1995, abandoned.

[51] **Int. Cl.<sup>7</sup>** ..... **B05D 3/04**; B05D 1/36; B05D 7/22

[52] **U.S. Cl.** ..... **427/142**; 427/140; 427/239; 427/248.1; 427/255.26; 427/255.4; 427/335; 427/337; 427/405; 427/419.7

[58] **Field of Search** ..... 427/230, 239, 427/248.1, 238, 405, 419.7, 335, 140, 142, 255.1, 255.26, 255.4, 337

## References Cited

### U.S. PATENT DOCUMENTS

|           |         |                 |       |           |
|-----------|---------|-----------------|-------|-----------|
| 2,063,596 | 12/1936 | Feiler          | ..... | 196/133   |
| 2,263,366 | 11/1941 | Peck et al.     | ..... | 196/47    |
| 3,890,686 | 6/1975  | Caubet          | ..... | 29/196    |
| 4,013,487 | 3/1977  | Ramquist et al. | ..... | 148/16.5  |
| 4,015,950 | 4/1977  | Galand et al.   | ..... | 428/638   |
| 4,404,087 | 9/1983  | Reed et al.     | ..... | 208/48 AA |

|           |         |              |       |           |
|-----------|---------|--------------|-------|-----------|
| 4,507,196 | 3/1985  | Reed et al.  | ..... | 208/48 AA |
| 4,511,405 | 4/1985  | Reed et al.  | ..... | 106/15.05 |
| 5,139,814 | 8/1992  | Sugao        | ..... | 427/46    |
| 5,208,069 | 5/1993  | Clark et al. | ..... | 427/239   |
| 5,405,525 | 4/1995  | Heyse et al. | ..... | 208/133   |
| 5,406,014 | 4/1995  | Heyse et al. | ..... | 208/134   |
| 5,413,700 | 5/1995  | Heyse et al. | ..... | 585/444   |
| 5,575,902 | 11/1996 | Heyse et al. | ..... | 208/48 R  |
| 5,674,376 | 10/1997 | Heyse et al. | ..... | 208/135   |
| 5,676,821 | 10/1997 | Heyse et al. | ..... | 208/135   |
| 5,849,969 | 12/1998 | Heyse et al. | ..... | 585/483   |
| 5,866,743 | 2/1999  | Heyse et al. | ..... | 208/135   |

## FOREIGN PATENT DOCUMENTS

|            |         |                |   |
|------------|---------|----------------|---|
| 1604604    | 12/1981 | United Kingdom | . |
| WO92/15653 | 9/1992  | WIPO           | . |
| WO94/15898 | 7/1994  | WIPO           | . |

## OTHER PUBLICATIONS

King et al., The Production of Ethylene by the Decomposition of n-Butane; the Prevention of Carbon Formation by the Use of Chromium Plating, no date available.

Primary Examiner—Shrive Beck

Assistant Examiner—Michael Barr

Attorney, Agent, or Firm—Pennie & Edmonds LLP

## [57] ABSTRACT

A process for producing a metallic protective layer whereby a metal-containing plating, cladding, paint or other coating is applied to at least a portion of a reactor system and then contacted with a gaseous stream containing hydrocarbons, such as impure hydrogen, thereby producing a continuous and adherent metallic protective layer. The gaseous stream preferably comprises hydrogen, which may be recycled. A preferred embodiment of the invention is directed to touch-up procedures where a portion of an already protected reactor system is replaced or rewelded and the protective layer is formed as the replaced portion is brought on-stream.

**27 Claims, No Drawings**

## USING HYDROCARBON STREAMS TO PREPARE A METALLIC PROTECTIVE LAYER

This application is a file-wrapper-continuation of application Ser. No. 08/475,308, filed Jun. 7, 1995, now abandoned.

### FIELD OF THE INVENTION

The present invention is a novel process for preparing a metallic protective layer on a substrate such as steel using a hydrocarbon-containing stream, for example using an impure hydrogen stream. The process is especially applicable to touch-up situations where a portion of an already protected reactor system is being replaced or modified. The novel process of this invention can be applied to all or a portion of a reactor system that is used to convert hydrocarbons.

### BACKGROUND

It is known to form metallic protective layers on surfaces that are susceptible to carburization, for example on steel surfaces that are used in ultra-low sulfur reforming processes (see WO92/15653) and in other hydrocarbon conversion environments, such as hydrodealkylation (see WO94/15898). These patent applications teach the need for a separate cure step using pure hydrogen to form the metallic protective layer.

Unfortunately, unless there is a hydrogen plant nearby, obtaining pure hydrogen free of hydrocarbons is often difficult, and can be very costly. Moreover, when pure hydrogen is used, it is generally used in a once-thru manner. This is because hydrogen recycle is typically not possible, since most recycle gas compressors cannot handle low molecular weight gases, such as hydrocarbon-free hydrogen. To overcome this recycle problem, the pure hydrogen can be diluted with an inert gas (such as nitrogen). Then compression and recycle become doable. However, nitrogen is also difficult to obtain and costly. In summary, the need for once-thru hydrogen or adding an inert gas significantly adds to the cost of the cure step.

Yet the art for preparing and curing metallic protection layers teaches using a hydrogen stream that is free of hydrocarbons. For example, Heyse et al. in WO 92/15653 teach:

"The metallic coatings and, in particular, the paints are preferably treated under reducing conditions with hydrogen. Curing is preferably done *in the absence of hydrocarbons.*" (page 25, line 23-5, emphasis added.)

An almost identical teaching can be found in Heyse et al. WO 94/15898 on page 23, lines 5-7. Both these patent applications are incorporated herein by reference, especially with regard to useful coating materials and process conditions for curing.

With the known curing process, the start-up procedure, for example, after painting or applying a metal-containing coating to a steel substrate, includes:

1. Heating the reactor system to the cure temperature (typically between 600-1800° F.) in a hydrogen atmosphere;
2. Holding at the cure temperature under hydrogen for up to 3 days;
3. Cooling the reactor system; and only then
4. Beginning standard process start-up procedures.

The new process of this invention eliminates the first three of these steps; it uses "normal", "standard", or only slightly

modified start-up procedures—that is, start-up in the presence of feed—to form the metallic protective layer in-situ. It does not require a separate and time-consuming cure step using pure or hydrocarbon-free hydrogen. Thus, the new process reduces start-up times by up to three days and increases on-stream time.

The new process of this invention is especially useful for touch-up situations. For example, it may be used to form a metallic protective layer on a section of a furnace tube that needs replacement. The tube is brought off-line, then cut out and replaced with a new steel section. This section is coated or painted with a metal-containing coating, and then welded in place. As the tube comes on-stream and heats in the presence of hydrocarbon feed, the protective layer is formed in-situ.

### SUMMARY OF THE INVENTION

In one embodiment, the present invention is a method of forming a continuous and adherent metallic protective layer on a steel substrate using a gaseous stream that contains substantial amounts of hydrocarbon. The invention is especially useful in touch-up situations where a portion of an already-coated and protected reactor system is replaced or cut open and then resealed.

In one embodiment, the invention is a process for producing a metallic protective layer whereby a metal-containing plating, cladding, paint or other coating is applied to at least one surface of a reactor system. The coated surface is then contacted with a gaseous stream containing hydrocarbons thereby producing the metallic protective layer. The hydrocarbon contacting step occurs before the adherent metallic protective layer is formed or fully cured.

In another embodiment, the invention is applied to a portion of a reactor system used to convert hydrocarbons. Here feed hydrocarbons are converted to desired products in a reactor system of improved resistance to carburization and metal dusting, wherein a metallic carburization-resistant protective layer has been produced on at least a portion of the reactor system, the improvement comprising producing said protective layer by contacting a metal-containing plating, cladding, paint or other coating with a gaseous stream containing hydrocarbons to produce the metallic protective layer.

It is preferred that the hydrocarbon-containing stream also contains hydrogen, that is, the contacting is done in a reducing environment. One preferred hydrocarbon-containing stream is the feed for the hydrocarbon conversion process including feed hydrogen. Another is impure hydrogen.

Among other factors this invention is based on the discovery that, contrary to the teachings of the art, the presence of hydrocarbons during the cure step does not prevent formation of a uninterrupted protective layer. Prior to this invention, it was believed that the presence of hydrocarbons and the interaction of these hydrocarbons with the coated metal or the steel surface would interfere with or adversely impact the formation of a continuous and adherent metallic protective layer.

This invention has significant advantages over other processes. It allows for simpler and less time consuming start-up procedures for the reactor system or a portion thereof, as it eliminates the need for a separate cure step using hydrocarbon-free hydrogen. It also allows for the use of inexpensive impure hydrogen streams or readily available feed streams to produce the protective coating. Additionally, impure hydrogen streams may be used once-thru without

significant cost penalties. Thus, the use of hydrocarbon-containing feeds for the cure step lowers the cost of preparing the protective layer. Moreover, the new process significantly simplifies the procedures for forming the protective layer, especially in touch-up situations.

#### DETAILED DESCRIPTION OF THE INVENTION

In one broad aspect, the present invention is a process which comprises forming a metallic protective layer on a base substrate, such as steel, in the presence of significant amounts of hydrocarbons. In a preferred embodiment, the protective layer is formed by contacting a metal-containing paint, preferably a reducible paint (such as a tin paint) with a stream containing hydrocarbons at temperatures and flow rates effective for converting the paint to a metallic protective layer.

Although the terms "comprises" or "comprising" are used throughout this specification, these terms are intended to encompass both the terms "consisting essentially of", and "consisting of" in various preferred aspects and embodiments of the present invention.

As used herein, the term "reactor system" is intended to include hydrocarbon conversion units that have one or more hydrocarbon conversion reactors, their associated piping, heat exchangers, furnace tubes, etc. Some of the preferred methods of hydrocarbon conversion where this invention is useful utilize catalysts that are sensitive to sulfur.

Here a sulfur converter reactor (for converting organic sulfur compounds to  $H_2S$ ) and a sulfur sorber reactor (for absorbing  $H_2S$ ) may also be present. These are included as part of the reactor systems when present.

As used herein, the term "metal-containing coating" or "coating" is intended to include claddings, platings, paints and other coatings which contain either elemental metals, metal oxides, organometallic compounds, metal alloys, mixtures of these components and the like. The metal(s) or metal compounds are preferably a key component(s) of the coating. Flowable paints that can be sprayed or brushed are a preferred type of coating.

#### Platings, Claddings, Paints and Other Coatings

Not all metal-containing platings, claddings, paints and other coatings are useful in this invention. Preferred metals are those that interact with, and preferably react with, the base material of the reactor system at temperatures below or at the intended hydrocarbon conversion conditions to produce an adherent metallic protective layer. The preferred metal depends on the hydrocarbon conversion process of interest, its temperatures, reactants, etc. Metals that are mobile or melt below or at the process conditions are especially preferred. These metals include those selected from among tin, antimony, germanium, arsenic, bismuth, aluminum, gallium, indium, copper, lead and mixtures, intermetallic compounds and alloys thereof. Preferred metal-containing coatings are selected from the group consisting of tin, antimony, germanium, arsenic, bismuth, aluminum, and mixtures, intermetallic compounds and alloys thereof. Especially preferred coatings include tin-, antimony- and germanium-containing coatings. These coatings all form continuous and adherent protective layers. Tin coatings are especially preferred—they are easy to apply to steel, are inexpensive and are environmentally benign.

Metal-containing coatings that are less useful include certain metal oxides such as molybdenum oxide, tungsten

oxide and chromium oxides. In part this is because it is difficult to form adherent metallic protective layers from these oxides using streams comprising hydrogen and hydrocarbons at most hydrocarbon processing conditions.

5 It is preferred that the coatings be sufficiently thick that they completely cover the base metallurgy and that the resulting protective layers remain intact over years of operation. This thickness depends on the intended use conditions and the coating metal. For example, tin paints may be applied to a (wet) thickness of between 1 to 6 mils, preferably between about 2 to 4 mils. In general, the thickness after curing is preferably between about 0.1 to 50 mils, more preferably between about 0.5 to 10 mils.

10 Metal-containing coatings can be applied in a variety of ways, which are well known in the art, such as electroplating, chemical vapor deposition, and sputtering, to name just a few. Preferred methods of applying coatings include painting and plating. Where practical, it is preferred that the coating be applied in a paint-like formulation (hereinafter "paint"). Such a paint can be sprayed, brushed, pigged, etc. on reactor system surfaces.

15 One preferred protective layer is prepared from a metal-containing paint. Preferably, the paint is a decomposable, reactive, metal-containing paint which produces a reactive metal which interacts with the steel. Tin is a preferred metal and is exemplified herein; disclosures herein about tin are generally applicable to other reducible metals such as germanium. Preferred paints comprise a metal component selected from the group consisting of: a hydrogen decomposable metal compound such as an organometallic compound, finely divided metal and a metal oxide, preferably a reducible metal oxide.

20 Some preferred coatings are described in WO 92/15653 to Heyse et al. This application also describes preferred paint formulations. One especially preferred tin paint contains at least four components or their functional equivalents: (i) a hydrogen decomposable tin compound, (ii) a solvent system, (iii) finely divided tin metal and (iv) tin oxide. As the hydrogen decomposable tin compound, organometallic compounds such as tin octanoate or neodecanoate are particularly useful. Component (iv), the tin oxide is a porous tin-containing compound which can sponge-up the organometallic tin compound, and can be reduced to metallic tin. 25 The paints preferably contain finely divided solids to minimize settling. Finely divided tin metal, component (iii) above, is also added to insure that metallic tin is available to react with the surface to be coated at as low a temperature as possible. The particle size of the tin is preferably small, for example one to five microns. Tin forms metallic stannides (e.g., iron stannides and nickel/iron stannides) when heated in streams containing hydrogen and hydrocarbons.

30 In one embodiment, there can be used a tin paint containing stannic oxide, tin metal powder, isopropyl alcohol and 20% Tin Ten-Cem (manufactured by Mooney Chemical Inc., Cleveland, Ohio). Twenty percent Tin Ten-Cem contains 20% tin as stannous octanoate in octanoic acid or stannous neodecanoate in neodecanoic acid. When tin paints are applied at appropriate thicknesses, typical reactor start-up conditions will result in tin migrating to cover small regions (e.g., welds) which were not painted. This will completely coat the base metal. Preferred tin paints form strong adherent protective layers early during the start-up process.

35 40 45 50 55 60 65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270 8275 8280 8285 8290 8295 8300 8305 8310 8315 8320 8325 8330 8335 8340 8345 8350 8355 8360 8365 8370 8375 8380 8385 8390 8395 8400 8405 8410 8415 8420 8425 8430 8435 8440 8445 8450 8455 8460 8465 8470 8475 8480 8485 8490 8495 8500 8505 8510 8515 8520 8525 8530 8535 8540 8545 8550 8555 8560 8565 8570 8575 8580 8585 8590 8595 8600 8605 8610 8615 8620 8625 8630 8635 8640 8645 8650 8655 8660 8665 8670 8675 8680 8685 8690 8695 8700 8705 8710 8715 8720 8725 8730 8735 8740 8745 8750 8755 8760 8765 8770 8775 8780 8785 8790 8795 8800 8805 8810 8815 8820 8825 8830 8835 8840 8845 8850 8855 8860 8865 8870 8875 8880 8885 8890 8895 8900 8905 8910 8915 8920 8925 8930 8935 8940 8945 8950 8955 8960 8965 8970 8975 8980 8985 8990 8995 9000 9005 9010 9015 9020 9025 9030 9035 9040 9045 9050 9055 9060 9065 9070 9075 9080 9085 9090 9095 9100 9105 9110 9115 9120 9125 9130 9135 9140 9145 9150 9155 9160 9165 9170 9175 9180 9185 9190 9195 9200 9205 9210 9215 9220 9225 9230 9235 9240 9245 9250 9255 9260 9265 9270 9275 9280 9285 9290 9295 9300 9305 9310 9315 9320 9325 9330 9335 9340 9345 9350 9355 9360 9365 9370 9375 9380 9385 9390 9395 9400 9405 9410 9415 9420 9425 9430 9435 9440 9445 9450 9455 9460 9465 9470 9475 9480 9485 9490 9495 9500 9505 9510 9515 9520 9525 9530

amounts up to one third Fe/Sn by weight. The addition of iron can, for example, be in the form of  $\text{Fe}_2\text{O}_3$ . The addition of iron to a tin containing paint should afford noteworthy advantages; in particular: (i) it should facilitate the reaction of the paint to form iron stannides thereby acting as a flux; (ii) it should dilute the nickel concentration in the stannide layer thereby providing better protection against coking; and (iii) it should result in a paint which affords the anti-coking protection of iron stannides even if the underlying surface does not react well.

#### Hydrocarbon-Containing Streams

Streams containing hydrocarbons are used to form the protective layer on the metal surfaces of the reactor system. One useful stream is impure hydrogen (e.g., hydrogen containing methane). Impure hydrogen streams are often available in refineries and chemical plants. They typically contain at least 1 volume % hydrocarbons, often 10% or more. Impure hydrogen is a low value stream which is often used as fuel. I have now discovered that these impure streams can be used to prepare an adherent and continuous metallic protective layer. Examples of two such streams are shown in the following table:

| Component                 | Stream 1 | Stream 2 |
|---------------------------|----------|----------|
| Hydrogen, vol %           | 20       | 88       |
| Methane, vol %            | 35       | 3        |
| Ethane, vol %             | 10       | 3        |
| Other hydrocarbons, vol % | 35       | 6        |

Stream 1 is a typical fluid catalytic cracker (FCC) fuel gas composition. Stream 2 is a typical fuel gas from a catalytic reformer. Although not required, in one preferred embodiment the non-hydrocarbon impurities in the gaseous stream are minimized. For example,  $\text{H}_2\text{S}$ , water, and organic sulfur-, oxygen- and nitrogen-containing compounds are removed.

Another stream that can be used to form the protective layer is hydrocarbon feed, including for example recycle hydrogen, such as that used in the process for which the protective layer is needed. The hydrocarbon in this stream is preferably selected from among hydrocarbons including naphthenes, paraffins, aromatics, alkylaromatics, olefins and light gases, including methane. Paraffinic streams are preferred. Hydrocarbon-containing streams may be combined or mixed with other gases such as carbon monoxide, and nitrogen. It is important that the cure stream be selected so that it not damage or attack the protective layer. Therefore, the preferred stream varies with the particular type of metal-containing coating being used. For example, halogen-containing streams are detrimental to some metallic coatings. One especially preferred stream comprises dry hydrocarbon feed or product combined with hydrogen.

An especially preferred stream is a mixture of hydrocarbon and hydrogen containing between about 1 to 90 volume percent hydrocarbon in hydrogen, preferably at least 10 volume percent hydrocarbon in hydrogen, more preferably containing between about 15 and 40 volume percent hydrocarbon. For example, a fixed bed catalytic reformer feed stream is useful. It typically has a hydrogen to hydrocarbon mole ratio of between about 3:1 and 10:1. Although not required, it is preferred to recycle the hydrogen stream, as it significantly reduces costs. With hydrocarbons present in the hydrogen, the recycle gas compressor will operate within design parameters.

Although not currently well understood, it appears that coatings prepared using hydrocarbon-containing streams and/or sulfur compounds produce protective layers that are about 50 percent thicker than those prepared in pure hydrogen. These thicker layers are expected to increase the protection afforded to the base substrate.

#### Cure Process Conditions

The cure step of this invention contacts a coated steel with a gaseous hydrocarbon-containing stream, such as feed, product, or impure hydrogen at elevated temperatures. Cure conditions depend on the coating metal and are selected so they produce a continuous and uninterrupted protective layer which adheres to the steel substrate. Contacting with the gaseous hydrocarbon-containing stream occurs while the protective layer is being formed. A prior cure step using pure hydrogen is not needed. The resulting protective layer is able to withstand repeated temperature cycling, and does not degrade in the reaction environment. Preferred protective layers are also useful in oxidizing environments, such as those associated with coke burn-off. In a preferred embodiment the cure step produces a metallic protective layer bonded to the steel through an intermediate bonding layer, for example a carbide-rich bonding layer.

Cure conditions depend on the particular metal coating as well as the hydrocarbon conversion process to which the invention is applied. For example, gas flow rates and contacting time depend on the cure temperature, the coating metal and the components of the coating composition. Cure conditions are selected so as to produce an adherent protective layer. In general, the process of this invention contacts the reactor system having a metal-containing coating, plating, cladding, paint or other coating applied to a portion thereof with the hydrocarbon-containing gas for a time and at a temperature sufficient to produce a metallic protective layer. These conditions may be readily determined. For example, coated coupons may be heated in the presence of the hydrocarbon-containing gas in a simple test apparatus; the formation of the protective layer may be determined using petrographic analysis.

It is preferred that cure conditions result in a protective layer that is firmly bonded to the steel. This may be accomplished, for example, by curing the applied coating at elevated temperatures. Metal or metal compounds contained in the paint, plating, cladding or other coating are preferably cured under conditions effective to produce molten or mobile metals and/or compounds. Thus, germanium and antimony paints are preferably cured between 1000° F. and 1400° F. Tin paints are preferably cured between 900° F. and 1100° F. Curing is preferably done over a period of hours, often with temperatures increasing over time. Preferred metallic protective layers, such as those derived from paints, are preferably produced under reducing conditions. Reduction/curing is preferably done at elevated temperatures in the presence of hydrocarbon streams containing hydrogen. The presence of hydrogen is especially advantageous when the paint contains reducible oxides and/or oxygen-containing organometallic compounds.

As an example of a suitable paint cure for a tin paint, the system including painted portions can be pressurized with flowing nitrogen, followed by the addition of a hydrocarbon-containing stream such as a 1:1 hydrogen/naphtha. The reactor inlet temperature can be raised to 800° F. at a rate of 50–100° F./hr. Thereafter the temperature can be raised to a level of 950–975° F. at a rate of 50° F./hr, and held within that range for about 48 hours.

In one embodiment of this invention the metallic protective layer be produced during plant start-up. However, when catalysts are present, it is important that the cure procedures do not result in poisoning of the catalyst or plugging of the catalyst pores. The utility of this process therefore depends in part on the location of, or presence of, a catalyst in the reactor system, and the catalyst's sensitivity towards the coating metal. The process of this invention is preferably applied to furnace tubes, heat exchangers, piping, etc., that are not adjacent to or immediately prior to catalyst beds.

If catalyst poisoning is a concern, provision should be made to prevent stray metal from contacting the catalyst. For example, the curing may be done prior to catalyst loading, or the catalyst may be removed for the curing step. Alternatively, catalyst may be present and a sorber or collector for stray metal, such as a high surface area alumina or silica guard bed, may be used upstream of the catalyst bed. In one embodiment, after the cure step, fresh hydrocarbon conversion catalyst or catalyst removed from the reactors is introduced into the reactor system.

#### The Base Construction Material

There are a wide variety of base construction materials to which the process of this invention may be applied. In particular, a wide range of steels may be used in the reactor system. In general, steels are chosen so they meet minimum strength and flexibility requirements needed for the intended hydrocarbon conversion process. These requirements in turn depend on process conditions, such as operating temperatures and pressures.

Useful steels include carbon steel; low alloy steels such as 1.25, 2.5, 5, 7, and 9 chrome steel; stainless steels including 316 SS and the 340 stainless steels such as 346; heat resistant steels including HK-40 and HP-50, as well as treated steels such as aluminized or chromized steels. The steel preferably contains iron and chromium in the zero oxidation state.

Depending on the components of the metal-containing coating, reaction of the reactor system metallurgy with the coating can occur. Preferably, the reaction results in an intermediate carbide-rich bonding or "glue" layer that is anchored to the steel and does not readily peel or flake. For example, metallic tin, germanium and antimony (whether applied directly as a cladding or produced in-situ) readily react with steel at elevated temperatures to form a bonding layer as is described in WO 94/15898 or WO 94/15896, both to Heyse et al.

#### Preferred Applications

The present invention for preparing a metallic protective layer can be utilized to protect one or more large portions of a reactor system, or only a small section thereof. In a preferred embodiment, the present invention is used to touch up relatively small areas of the reactor system that already have a metallic protection layer applied thereto. For example, it may be necessary to replace a portion of the reactor system, due to a failure or a change in process configuration. For example, a section of a furnace tube or reactor screen may need replacement. Here, the furnace tube or section of the tube is isolated or brought off-line. A replacement tube or section is then coated with a metal-containing coating, plating, cladding or paint. The coated tube is then put on-stream in the presence of feed, without a separate cure step. The coating cures in-situ to produce the protective layer.

It is also envisioned that this invention would be especially useful for providing protective layers on new, replace-

ment parts for the reactor internals (such as screens, distributors, associated piping, center pipe and its screens) should they require replacement, and for forming protective layers on transfer piping, flanges and nozzles which are newly constructed or rewelded.

#### Application to Hydrocarbon Conversion Processes

Reactor systems having metallic protective layers prepared by the novel process of the invention are effective in reducing coking and/or carburization in a variety of hydrocarbon conversion processes. Thus, the novel process of this invention for producing a protective layer can be applied to all or a portion of a reactor system used for converting hydrocarbons.

Preferred hydrocarbon conversion processes include dehydrocyclization of C<sub>6</sub> and/or C<sub>8</sub> paraffins to aromatics; catalytic reforming; non-oxidative and oxidative dehydrogenation of hydrocarbons to olefins and dienes; dehydrogenation of ethylbenzene to styrene and/or dehydrogenation of isobutane to isobutylene; conversion of light hydrocarbons to aromatics; transalkylation of toluene to benzene and xylenes; hydrodealkylation of alkylaromatics to aromatics; alkylation of aromatics to alkylaromatics; production of fuels and chemicals from syngas (H<sub>2</sub> and CO); steam reforming of hydrocarbons to H<sub>2</sub> and CO; production of phenylamine from aniline; methanol alkylation of toluene to xylenes; and dehydrogenation of isopropyl alcohol to acetone. Preferred hydrocarbon conversion processes include dehydrocyclization, catalytic reforming, dehydrogenation, isomerization, hydrodealkylation, and conversion of light hydrocarbon to aromatics, e.g. Cyclar-type processing. Preferred embodiments include those where a catalyst, preferably a platinum catalyst, is used to dehydrogenate a paraffin to an olefin, or to dehydrocyclization a paraffinic feed containing C<sub>6</sub>, and/or C<sub>8</sub> hydrocarbons to aromatics (for example, in processes which produce benzene, toluene and/or xylenes).

The present invention is especially applicable to hydrocarbon conversion processes which require catalysts, especially noble metal catalysts containing Pt, Pd, Rh, Ir, Ru, Os, particularly Pt containing catalysts. These metals are usually provided on a support, for example, on carbon, on a refractory oxide support, such as silica, alumina, chlorided alumina or on a molecular sieve or zeolite. Preferred catalytic processes are those utilizing platinum on alumina, Pt/Sn on alumina and Pt/Re on chlorided alumina; noble metal Group VIII catalysts supported on a zeolite such as Pt, Pt/Sn and Pt/Re on zeolites, including L type zeolites, ZSM-5, SSZ-25, SAPO's, silicalite and beta.

In a preferred embodiment, the invention uses of a medium-pore size or large-pore size zeolite catalyst containing an alkali or alkaline earth metal and charged with one or more Group VIII metals. Especially preferred catalysts for use in this invention are Group VIII metals on large pore zeolites, such as L zeolite catalysts containing Pt, preferably Pt on non-acidic L zeolite. Useful Pt on L zeolite catalysts include those described in U.S. Pat. No. 4,634,518 to Buss and Hughes, in U.S. Pat. No. 5,196,631 to Murakawa et al., in U.S. Pat. No. 4,593,133 to Wortel and in U.S. Pat. No. 4,648,960 to Poepelmeir et al.

The present invention is especially applicable to hydrocarbon conversion processes that are operated in conjunction with sulfur removal processes or under reduced or low-sulfur conditions using a variety of sulfur-sensitive catalysts. These processes are well known in the art. These processes generally require some feed cleanup, such as hydrotreating

and/or sulfur sorption. They include catalytic reforming and/or dehydrocyclization processes, such as those described in U.S. Pat. No. 4,456,527 to Buss et al. and U.S. Pat. No. 3,415,737 to Kluksdahl; catalytic hydrocarbon isomerization processes such as those described in U.S. Pat. No. 5,166,112 to Holtermann; and catalytic hydrogenation/dehydrogenation processes.

In an especially preferred embodiment, the hydrocarbon conversion process is conducted under conditions of "low sulfur". In these low-sulfur systems, the feed will preferably contain less than 50 ppm sulfur, more preferably, less than 20 ppm sulfur and most preferably less than 10 ppm sulfur.

For systems using catalysts that are poisoned by sulfur, it is preferred that hydrocarbon sulfur levels are such that they do not significantly reduce catalyst performance. This level of sulfur depends on the specific catalyst. Generally it is preferred that the sulfur level be very low, i.e., below about 5 ppm, preferably below 1 ppm, and more preferably below 500 ppb. For highly sulfur-sensitive catalysts, sulfur levels should be ultra-low, i.e., below 100 ppb, preferably below 50 ppb, and more preferably below 10 ppb. These substantially sulfur-free gases are preferably also free of oxygen-containing and nitrogen-containing contaminants, such as  $\text{NH}_3$  or water.

Gases containing sulfur compounds and other contaminants can be treated to remove these contaminants. Those skilled in the art will appreciate that a variety of treatment methods, including hydrotreating, mild reforming and sorption processes, to name a few, are well known for this purpose.

To obtain a more complete understanding of the present invention, the following examples illustrating certain aspects of the invention are set forth. It should be understood, however, that the invention is not intended to be limited in any way to the specific details of the examples.

#### EXAMPLE 1

This experiment was done in a pilot plant using a  $\frac{1}{4}$ " O.D. reactor made of 316 stainless steel. The reactor was coated with a tin-containing paint. The paint consisted of a mixture of 2 parts powdered tin oxide, 2 parts finely powdered tin (1-5 microns), 1 part stannous neodecanoate in neodecanoic acid (20% Tin Tem-Cem) mixed with isopropanol, as described in WO 92/15653. The coating was applied to the inner surface of the tube by filling the tube with paint and letting the paint drain.

After drying, a hydrocarbon-containing stream containing 100 ppmv  $\text{H}_2\text{S}$ , 50 vol. % n-hexane and the balance hydrogen was provided at a flow rate of 50 standard cubic centimeters per minute at atmospheric pressure and room temperature. The reactor was then heated to about 1100° F. over 30 hours and held at this temperature for an additional 60 hours with gas flowing. Process gases were used in a once-thru manner.

After this procedure was completed, the reactor was cut open and the resulting layer was examined visually. The steel surface was substantially free of coke. Cross-sections of the steel were mounted in epoxy and polished. They were then examined using petrographic and scanning electron microscopy. The micrographs showed that the tin paint had reduced to metallic tin under these conditions. A continuous and adherent metallic (iron/nickel stannide) protective layer having a thickness of about 30 microns was observed on the steel surface.

#### EXAMPLE 2

The procedure of Example 1 was repeated using a gas containing 35 volume percent of n-hexane and the balance

hydrogen. No sulfur was added. As in Example 1, a continuous and adherent metallic protective layer was produced on the steel surface.

While the invention has been described above in terms of preferred embodiments, it is to be understood that variations and modifications may be used as will be appreciated by those skilled in the art. Indeed, there are many variations and modifications to the above embodiments which will be readily evident to those skilled in the art, and which are to be considered within the scope of the invention as defined by the following claims.

What is claimed is:

1. A touch-up process for a producing a metallic protective layer, comprising,
  - (a) providing a first metallic protective layer to a portion of a reactor system;
  - (b) reacting hydrocarbons in said reactor system;
  - (c) applying a metal-containing paint or coating to at least one surface of the reactor system as a touch-up;
  - (d) thereafter contacting said surface with a gaseous stream containing hydrogen and at least 10 volume percent hydrocarbons, thereby producing a continuous and adherent metallic protective layer.
2. The touch-up process of claim 1 wherein the gaseous stream is fuel gas or impure hydrogen.
3. The touch-up process of claim 1 wherein the metal-containing coating contains a metal selected from the group consisting of tin, antimony, germanium, arsenic, bismuth, aluminum, gallium, indium, copper, lead, and mixtures, intermetallic compounds and alloys thereof.
4. The touch-up process of claim 1 wherein the metal-containing coating contains a metal selected from the group consisting of tin, antimony and germanium.
5. The touch-up process of claim 1 wherein the metal-containing coating comprises a tin paint.
6. The touch-up process of claim 1 wherein the metallic protective layer comprises iron stannide.
7. The touch-up process of claim 1 wherein the gaseous stream contains methane.
8. A method for producing a metallic protective layer on a replacement portion of a reactor system, comprising,
  - replacing an existing portion of a reactor system with a replacement portion;
  - applying a metal-containing plating, cladding, paint or other coating to said replacement portion; and
  - operating said reactor system using a gaseous stream containing hydrogen and at least 10 volume percent hydrocarbons to cure said metal-containing plating, cladding, paint or other coating and thereby produce a metallic protective layer on said replacement portion.
9. The method of claim 8, wherein said metal-containing plating, cladding, paint or other coating comprises a metal selected from the group consisting of tin, antimony, germanium, arsenic, bismuth, aluminum, gallium, indium, copper, lead, and mixtures, intermetallic compounds and alloys thereof.
10. The method of claim 8, wherein said metal-containing plating, cladding, paint or other coating comprises a metal selected from the group consisting of tin, antimony and germanium.
11. The method of claim 8, wherein said metal-containing plating, cladding, paint or other coating comprises a tin paint.
12. The method of claim 8, wherein said gaseous stream is impure hydrogen or fuel gas.
13. The method of claim 8, wherein said gaseous stream is hydrocarbon feed to said reactor system.

## 11

14. The method of claim 13, wherein said hydrocarbon feed is a paraffinic stream.
15. The method of claim 13, wherein said hydrocarbon feed further comprises carbon monoxide.
16. The method of claim 13, wherein said hydrocarbon feed further comprises nitrogen.
17. The method of claim 8, wherein said gaseous stream comprises approximately 15–40 volume percent hydrocarbons.
18. The method of claim 8, wherein said gaseous stream comprises methane.

19. The method of claim 8, wherein said metallic protective layer comprises iron stannide.
20. The method of claim 8, wherein said operating step further comprises the step of operating said reactor system under typical start-up conditions to cure said metal-containing plating, cladding, paint or other coating.

21. The method of claim 8, wherein said operating step further comprises the step of operating said reactor system under typical operating conditions to cure said metal-containing plating, cladding, paint or other coating.

22. The method of claim 8, wherein said replacement portion comprises a portion of a furnace tube.

23. A method for producing a metallic protective layer on a replacement portion of a reactor system, comprising, replacing an first existing portion of a reactor system with a replacement portion, wherein said reactor system has a second existing portion with a previously formed metallic protective layer adjacent to said first existing portion;

25

## 12

applying a metal-containing plating, cladding, paint or other coating to said replacement portion; and operating said reactor system using a gaseous stream containing hydrogen and at least 10 volume percent hydrocarbons to cure said metal-containing plating, cladding, paint or other coating and thereby produce a metallic protective layer on said replacement portion that is contiguous with said previously formed metallic protective layer.

24. A method for producing a metallic protective layer on a replacement portion of a reactor system, comprising, charging a reactor system with a catalyst; replacing an existing portion of said reactor system with a replacement portion; applying a metal-containing plating, cladding, paint or other coating to said replacement portion; and operating said reactor system using a gaseous stream containing hydrogen and at least 10 volume percent hydrocarbons to cure said metal-containing plating, cladding, paint or other coating and thereby produce a metallic protective layer on said replacement portion while keeping said catalyst in said reactor system.

25. The method of claim 24, wherein said catalyst is a sulfur-sensitive catalyst.

26. The method of claim 24, wherein said gaseous stream has approximately less than 5 ppm sulfur.

27. The method of claim 26, wherein said gaseous stream has approximately less than 10 ppb sulfur.

\* \* \* \* \*